

## UNITED STATES PATENT OFFICE.

CLARENCE RUDOLPH REIERSON, OF HAVRE, MONTANA.

## SOLUTION FOR TREATING PHOTOGRAPHS AND PROCESS OF PREPARING THE SAME.

No Drawing. Original application filed August 2, 1922, Serial No. 579,244. Divided and this application filed October 25, 1923. Serial No. 670,715.

To all whom it may concern:

Be it known that I, CLARENCE RUDOLPH REIERSON, a citizen of the United States, residing at Havre, in the county of Hill 5 and State of Montana, have invented new and useful Improvements in Solutions for Treating Photographs and Processes of Preparing the Same, of which the following is a specification.

10 This invention relates to the decoration of photographs and pertains particularly to a liquid preparation used in the production of oil colored photographs. Among other features the invention is directed to the use 15 of particular materials and to the steps in the process by which the materials are prepared. The particular sequence in which the materials are used in coloring photographs with oil colors is claimed in my co- 20 pending application Serial No. 579,244, filed August 2, 1922, from which this application has been divided.

One purpose of the invention is to reduce the time necessary to complete the application of oil colors to a photographic print. Another purpose is to make possible a more even blending of oil colors than has heretofore been known. Another purpose is to provide a lustrous finish for photographic prints without destroying the soft tone of the print. Finally the invention 30 enables the artist to work rapidly without the smearing of oil colors, and makes it possible to complete the work in a remarkably short time.

Heretofore to complete the coloring of an average sized photographic print it has not been possible in less than from one to three hours, and after the completion of 40 the coloring step two or three days have been usually required to properly dry the work. The details of the present invention enable the average artist to color with oil paint a photograph in fifteen or twenty 45 minutes, and the work thus completed will dry within seven to ten hours. Thus a dozen photographs could be colored in oil in one evening, and could be dry by morning, when they are in condition for mounting and delivery to the purchaser.

The invention includes three chief essential features which are as follows.

First, the materials and the process of preparing the materials into a composition

for application directly to the photographic 55 print. This is the present invention.

Second, the process of preparing the photographic print with the completed material of the first feature in order to make the print ready for receiving the decorative 60 paint coating. This is the invention of my application, Serial No. 579,244, filed August 2, 1922, from which this has been divided.

Third, the materials and the process of 65 preparing the mixture of the same for the outer and final protective coating which is applied to the decorative paint coats. This was originally claimed in my application, 70 Serial No. 579,244, filed August 2, 1922.

The details of these three features will now be described.

The first feature, which includes the preparation and materials for the initial treating material, relates to a liquid which, when 75 properly applied, produces an oil body surface upon the dried emulsion of photographic prints, which surface is suitable for the reception and blending thereon of artists' oil colors such as are usually sold in 80 tubes.

To make the liquid of feature one, the following ingredients in the following proportions, are mixed in accordance with the steps specified. 3 parts of raw linseed oil, 85 3 parts of japan drier, and 2 parts of commercial ether are used. The japan drier is added to the oil and thoroughly mixed. To the resultant product the specified proportion of ether is added, and the resultant 90 material is thoroughly mixed. Care should be taken to use substantially the proportions and sequence specified because a perfectly acting solution may be prepared in this way, but if the proportions and order 95 of treatment are materially disregarded, undesirable precipitates may be formed and the materials spoiled.

The treatment of the photographic print should be conducted substantially according to the following details. The solution prepared in accordance with feature one, should be applied to the dried emulsion which is the surface of the print with a tuft of cotton or some other equally soft material, and any surplus solution, which has not been absorbed by the emulsion on the print must be removed by rubbing the 100 105

damp surface with a piece of dry soft cotton fabric. The solution acts upon the dried photographic emulsion of the print in substantially the following manner. The 5 ether of the solution permits the introduction into the dried emulsion of the print of the required quantity of oil and japan drier. Probably the action is one in which the ether opens the pores of the dried emul- 10 sion, or otherwise so prepares it, so as to permit the introduction of the oil and drier, or at least permits a unified combination of the oil and drier with the material of the dried emulsion. The ultimate effect, re- 15 gardless of the theory of the action, is that the material sizes the dried emulsion, or so prepares it, as to make possible the application and blending thereon of artists' oil colors in tubes evenly, smoothly, and 20 without smearing, all to a degree of per- fection heretofore not possible before the use of the particular solution mentioned. When oil colors are applied to a print or to a dried emulsion to which oil has been 25 applied in a manner different from the above described, the application of the ma- terial is not even or smooth, the oil rubs off and smears, and the oil colors also tend to rub off and smear. 30 The japan drier, probably augmented by the action of the ether, serves to make pos- sible unusual rapidity on the part of the artist who is applying the oil colors because the artist is enabled to have the oil colors 35 under control at all times, and also because the completed work dries rapidly. The dry- ing qualities are just such as to cause the colors to take hold without running or smearing, and yet the colors do not set 40 so rapidly as to take the control of the work out of the artist's hands.

Feature three, relating to the protecting coating, will now be described. This ma- 45 terial is intended for use as a protective lustre producing material for application directly over the oil colored photograph. The object of this feature of the invention is to provide a liquid, which when properly applied to a completed oil colored photo- 50 graph, adds the desired lustre and gives to it an unnoticeable, even, protective cover- ing. To make this solution 5 parts of raw linseed oil and 1 part of japan drier are thor- 55oughly mixed. The material is applied to the decorative paint coat on the photo- graphic print by the use of a tuft of cotton, and any surplus solution must be removed by rubbing gently with a similar dry tuft of cotton. The effect of the application of 60 the protective coating is the production of a rapidly drying, unnoticeable coating which protects against dust, dirt, and the fading of the color coat. The desired lustre may thus be added to the completed work 65 of the color coat without destroying the

softer tones of the colored photograph. The same advantageous results obtained by using the protective coat may be accomplished by using the solution upon black and white, or sepia prints, as have been described by using 70 the material over prints finished in oil colors.

The various features of this invention may be used, and the materials of each of the solutions may be applied effectively, in 75 the treatment of matt, semi-matt, or gloss photographic prints, as well as in the making of Doretypes.

By following the details of the present invention a photographic print may be col- 80 ored and the coloring protected so that the final product has such a perfect blending of color that the lines of the colors and the material of the protective coat are im- perceptible. In addition to the proper 85 blending, the time for the coloring is re- duced to one-fifth to one-eighth of the time ordinarily required prior to the use of the initial treatment solution.

I claim:—

1. The process of preparing a liquid coat- 90 ing composition for treating photographic prints to prepare such prints for the recep- tion of oil paints which process comprises thoroughly mixing japan drier and linseed 95 oil, and adding to the resultant mixture ether and thoroughly mixing the resultant solution.

2. The process of preparing a liquid coat- 100 ing composition for treating photographic prints which comprises thoroughly mixing 3 parts japan drier with 3 parts of raw lin- seed oil, and adding to this mixture 2 parts of ether and thoroughly mixing the re- sultant solution.

3. A liquid coating composition for treat- 105 ing photographic prints to prepare such prints for the reception of oil paints which composition consists entirely of a mixture of raw linseed oil, a liquid drier, and ether.

4. A liquid coating composition for treat- 110 ing photographic prints to prepare such prints for the reception of oil paints which composition consists entirely of a mixture of linseed oil, japan drier, and ether.

5. A liquid coating composition for treat- 115 ing photographic prints to prepare such prints for the reception of oil paints which composition consists entirely of a mixture of raw linseed oil, japan drier, and ether.

6. A liquid coating composition for treat- 120 ing photographic prints which composition comprises a mixture of raw linseed oil, japan drier, and ether in the proportion of 3 parts of linseed oil, 3 parts of drier and 125 2 parts of ether.

In testimony whereof I affix my signa- ture.

CLARENCE RUDOLPH REIERSON.